

# UNITED STATES PATENT OFFICE.

HENRY R. WARDELL, OF NEW YORK, N. Y., ASSIGNOR TO H. W. JOHNS-MANVILLE COMPANY, A CORPORATION OF NEW YORK.

## ROAD SURFACE AND PRESERVATIVE.

1,058,503.

Specification of Letters Patent.

Patented Apr. 8, 1913.

No Drawing.

Application filed July 16, 1912. Serial No. 709,790.

*To all whom it may concern:*

Be it known that I, HENRY R. WARDELL, a citizen of the United States of America, residing at New York city, borough of Manhattan, county and State of New York, have invented certain new and useful Improvements in Road Surfaces and Preservatives, of which the following is a specification.

My invention relates to compositions for 10 surfacing, repairing and preserving a smooth surface on roads.

It comprises an improved asphaltic base oil artificially produced which is easily applied to the road surface and soon forms a solid asphalt cement, compacting and solidifying the mineral content of the roadbed and forming a smooth, solid surface thereon.

Heretofore it has been customary to use 20 residual oils for surfacing roads, which oils are produced by distilling the lighter constituent from the crude oils obtained from Oklahoma, Kansas, Illinois and Ohio, or other native oils. The constituents usable as kerosene, naphtha and the like are distilled 25 over from these natural oils until the residuum has a density of from 13 to 24 degrees Baumé, and this residuum is used for road surfacing. The base of this oil is not asphaltic, but is a greasy sludge, not cementitious in its nature. The oily constituents of 30 this natural residuum are not volatile and evaporate slowly if at all under exposure to the atmosphere. They remain on the road surface for weeks and months, forming an emulsion with the sand and dust particles, thereby creating a greasy mixture of mud, and semifluid oil which is a source of danger 35 to vehicles and disgust to pedestrians. Practically the only beneficial result of the use of 40 this natural oil residuum is to lay the dust. Otherwise the road bed is little improved by its use.

I have discovered that if a true asphaltic 45 base oil be produced by dissolving natural solid asphaltic materials in a volatile vehicle such as naphtha, and applied to the road surface, the vehicle will practically volatilize in less than 48 hours, leaving the solid asphaltic base intimately mingled with the sand, gravel or broken stone of the road bed, and forming a firmly cemented smooth 50 surface which is free from dust. The surface layer thus formed is as tenacious, efficient and durable as an ordinary asphalt 55 pavement.

Among the characteristic features of my invention are, first, a solid base of natural asphalt, second, a solvent comprising a true asphaltic base oil, and third, a volatile vehicle which holds the other elements in solution until they have been evenly distributed over the road surface and incorporated with the mineral content thereof to form a solidly cemented surfacing sheet after the vehicle has evaporated.

The best formula embodying my invention at present known to me, and the preferred process of making, compounding and using the same, according to my present information, is as follows: I take: 1 part by 60 weight of Trinidad manjack; 1 part by weight of gilsonite; 2 parts by weight of hydrolene, which is a residual pitch derived from the distillation of Texas oil; 8 $\frac{1}{4}$  parts by weight of Texas oil, known as mosaic oil, which has a density of about 13 degrees Baumé. These may be mixed by heating 65 and stirring and when mixed in the above stated proportion will form an asphaltic base compound having a consistency represented on a standard penetrating machine by a penetration of 112 at a temperature of 77 degrees Fahrenheit. To this base, while 70 warm, I add from 3 $\frac{1}{4}$  to 4 $\frac{1}{2}$  parts of naphtha and incorporate by stirring. This produces 75 an artificial, asphaltic base oil, of a density of from 13 to 23 degrees Baumé, (according to how much naphtha is used) which has much the same appearance as the natural 80 residuum heretofore used for road surfacing purposes. My artificially produced oil, however, has the advantages due to the fact that it is composed of a solution of materials having the extreme characteristics of a solid, 85 cementitious asphaltic body on the one hand and a light, highly volatile vehicle on the other; while the natural residuum heretofore used has little real asphaltic content, and little really volatile oil, being mainly 90 composed of intermediate oils and sludges which will neither volatilize nor solidify 95 under atmospheric conditions, but persist in the form of a greasy slime.

The artificial oil so produced is applied to the surface of the road by pouring from 100 a pot or tank, using about a gallon to the square yard of surface, in the usual manner, the same as natural oils are applied. The material must be at a temperature sufficient 105 to give it the desired fluidity to run easily 110

and evenly. If  $4\frac{1}{2}$  parts of naphtha are used the product is sufficiently fluid at summer temperature, say 77 degrees Fahrenheit. If only  $3\frac{1}{4}$  parts of naphtha are used, 5 the product should be heated to a temperature of from 160° to 200 degrees Fahrenheit to give it the needed fluidity. The material thus applied at or near atmospheric temperature produces quite as rapid a cement- 10 ing action on the mineral content as would ordinary asphalt applied at the higher temperatures necessary for melting it. Thus considerable saving of expense results in that the heating of the material may be en- 15 tirely omitted or carried on only to a low degree.

By the term "naphtha," herein used, I mean the densest of the hydrocarbon fluids volatilizing by exposure to the atmosphere. 20 It is the commercial product which is lighter than fuel oil, but denser than benzine or gasolene. This serves as a solvent or vehicle in which the pure asphaltic base is suspended so as to permit its even application 25 to the road surface. If the road is wet the naphtha also serves to "cut" into the moisture on the surfaces of the mineral particles and so insure their firm adhesion to the cementing body formed by the asphalt content. The naphtha entirely evaporates in about 48 hours, leaving the asphalt base firmly binding the mineral content of the road surface together in a smooth solid body practically the same thing as a good 30 asphalt pavement, which maintains the qualities of hardness and toughness in both

winter and summer. The resultant road surface can of course be improved by adding a top dressing of clean sand, gravel or stone screenings, in the usual way, immediately 40 after application of my compound to the road bed.

While I have given above the formula best adapted to carry out my invention, other combinations of natural asphalt and 45 asphaltic base oils might be used and suspended in other volatile vehicles besides those before mentioned, to produce my improved result to a less perfect degree, so long as the liquid vehicle was sufficiently 50 volatile to pass off in a short time, and the asphalt base sufficiently stable and cementitious to form a hard, tough and durable road surface out of the mineral particles of the road bed incorporated therewith. 55

Having, therefore, described my invention, I claim:

1. A road surfacing composition comprising natural solid asphalt dissolved in an asphaltic base oil and suspended in a volatile liquid vehicle. 60

2. A road surfacing composition comprising one part of Trinidad manjack, one part of gilsonite and two parts of hydrolene, dissolved in about eight parts of mosaic oil and 65 suspended in about three or four parts of naphtha.

HENRY R. WARDELL.

Witnesses:

ERNEST SEARING,  
J. S. CORRALL.